

# UNITED STATES PATENT OFFICE.

OTTO STRUENSEE, OF PHILADELPHIA, PENNSYLVANIA.

## COATING FOR FLONGS.

1,385,284.

Specification of Letters Patent. Patented July 19, 1921.

No Drawing.

Application filed September 22, 1920. Serial No. 412,021.

To all whom it may concern:

Be it known that I, OTTO STRUENSEE, a citizen of the United States, residing in Philadelphia, Pennsylvania, have invented 55  
5 Coating for Flongs, of which the following is a specification.

This invention relates to compositions particularly adapted for coating the surfaces of stereotype matrices, and one object 0 of this invention is to provide a coating of such a nature that it will perfectly fill the pores and enter all depressions,—no matter how minute, in the plate to be duplicated when the pulp to which it is applied 5 is properly pressed against it.

It is further desired that the coating shall be of such a nature as to attract rather than repel the molten metal of the casting and to present to the latter a perfectly smooth surface, which permits the flong being easily freed from said casting when this has sufficiently cooled.

Further, the invention contemplates a coating of such a nature as will fit it for use 25 in commercial stereotyping work, so as to make possible the satisfactory reproduction of half tones, in contradistinction to the coarser newspaper work commonly done, and it is also desired that the coating shall be of 30 such a nature as to completely penetrate and, as it were, amalgamate with the fibers of stereotype paper or pulp in order to impart to it the strength necessary to prevent its being injured by the high temperature of 35 the molten metal to which it is exposed.

In accordance with my invention the composition which I have invented consists of a mixture of ten parts air floated talc, two parts of pulverized corn flour, one half part 40 pulverized gum arabic, one half part of formaldehyde or any other preservative and about thirty parts of water. After these ingredients are intimately mixed, they are boiled until the liquid has a creamy consistency, when it is allowed to cool. 45

It may now be applied to the surface of the pulp or paper constituting a flong, prior to the application of the latter to a plate to be duplicated, either by being brushed on 50 or by being poured over the surface of said flong in such manner as to allow the surplus liquid to run off. While still in a plastic

state, the pulp matrix with its coating aforesaid is applied to the face of the plate to be duplicated and is dried and otherwise treated in the well known manner for the production of stereotyped molds. Owing to the peculiar composition and nature of my coating, the matrix may be easily freed or removed from the plate after being forced into intimate contact therewith, and when examined under the microscope is found to have perfectly received even the most minute variations in the surface of said plate, so that it is especially adapted for half tone 60 reproductions.

When molten metal is poured into the mold prepared as above, I have found that it wets or is attracted to the material of the coating, perfectly entering all the depressions and surface variations of the matrix without injuriously affecting the same, because said coating penetrates and completely fills the minute spaces between the fibers of the paper, and presents to the molten metal 75 a hard, smooth and unbroken face which gives to the matrix a long life and permits it to be used for a number of reproductions or castings.

While I preferably use air floated talc as the principal ingredient of my coating compound, other equivalent substances such as china clay or kaolin may be used without departing from my invention, although they do not give as good results since they lack 80 the fine division and other characteristic qualities of the talc and to a greater or less extent repel molten stereotype metal. Likewise while I preferably use finely pulverized corn flour, it is possible to employ other substances such as rice starch, but again this 85 does not give as satisfactory results as I have found produced by corn flour. In place of the gum arabic, dextrin or other suitable adhesive material may be employed.

I claim:—

1. A coating for stereotype matrices containing a finely divided base material having the characteristic of attracting molten stereotype metal; a starchy material; an adhesive; with a suspending liquid. 100

2. A coating for stereotype matrices containing a finely divided base material having the characteristic of attracting molten

stereotype metal; a starchy material; an adhesive; a suspending liquid; and a preservative.

3. A coating for stereotype matrices containing air-floated talc; starchy material; and an adhesive.

4. A coating for stereotype matrices containing talc; corn flour; and an adhesive material.

10 5. A coating for stereotype matrices containing approximately twenty parts of finely divided talc; four parts of corn flour; and one part of an adhesive.

15 6. A coating for stereotype matrices containing approximately twenty parts of finely

divided talc; four parts of corn flour; one part of an adhesive; with sixty parts of water.

7. A coating for stereotype matrices containing approximately twenty parts of finely 20 divided talc; four parts of corn flour; one part of an adhesive; sixty parts of water; with one part of formaldehyde.

8. A coating for stereotype matrices consisting of a creamy liquid containing ap- 25 proximately twenty parts of air floated talc; four parts of corn flour; one part of gum arabic and one part of a preservative.

OTTO STRUENSEE.